

March 15, 1938.

W. N. MAYO

2,111,219

AUTOMOTIVE VEHICLE DASH HEAT AND SOUND INSULATION

Filed March 6, 1936

INVENTOR.  
William N. MayoBY  
Barnea, Kuselle, Laughlin & Raisch  
ATTORNEY.S

## UNITED STATES PATENT OFFICE

2,111,219

AUTOMOTIVE VEHICLE DASH HEAT AND  
SOUND INSULATIONWilliam N. Mayo, Detroit, Mich., assignor to  
Zonolite Corporation of Michigan, Detroit,  
Mich., a corporation of Michigan

Application March 6, 1936, Serial No. 67,416

2 Claims. (Cl. 154—44)

This invention relates to automotive vehicle dash heat and sound insulation and more particularly to a heat and sound insulating board for this purpose.

5 It is customary in the manufacture of automotive vehicles to prevent the transmission of heat and noise from the motor through the body dash-board into the vehicle body. At present it is common practice to insulate the vehicle body dash by covering the inside face of the dash with a loosely felted or woven mat of jute or similar fibers. This jute mat is used primarily for sound absorption to prevent the transmission of motor noises through the dash into the body. The 10 jute or similar sound absorbing mat is covered by a compressed fiberboard, such as Celotex. This compressed wood fiberboard is used primarily as a heat insulator to prevent the transmission of the engine heat through the dash into the vehicle body. This compressed wood fiberboard is stiff and self-sustaining and therefore must be cut into a plurality of pieces to conform to the contour of the body dash. In some instances the jute mat, which is limp and not 15 self-sustaining, is cemented to the compressed wood fiberboard. The wood fiberboard is then covered by a decorative lining such as an embossed fiber and asphalt composition board which is thermoplastic and easily deformable to fit the 20 contour of the dash. The entire assembly of the jute mat, wood fiberboard, and fiber asphalt board is then bolted to the dash. This commonly used arrangement for heat and sound insulating the dash is not only cumbersome but 25 expensive.

It is the object of this invention to produce a board which is cheap, light in weight, and has excellent sound absorbing as well as heat insulating properties, and which in the making can be very easily formed to fit any contour desired, such as the contour of the vehicle dash.

In the drawing:

Fig. 1 is a section through the dash-board of an automotive vehicle showing the dash-board insulated with the board which is the subject matter of this invention.

Fig. 2 is an elevation of the board, and

Fig. 3 is a sectional view of the same.

50 The board 1, which is the subject matter of this invention, may be made from any soft fiber material 2 such as jute, hair, hair felt, felt, cotton fiber, felt corn products, wood fiber, sugar cane, and the various mineral wools and fibers.

55 These fiber materials are felted or woven in the

form of a mat or web. The jute or other fibrous web is soft and limp or flexible so that it is not self-sustaining but has good sound and some heat insulating properties. The thickness of the jute or other fibrous web will vary depending upon the uses to which it will be put.

5 Inasmuch as this type of jute or other fibrous web is limp and not self-sustaining, it must be stiffened or reinforced so that a jute or fibrous board is obtained which retains all of the desirable properties of a jute fiber web but which has the undesirable limp or flexible characteristic obviated. This object is obtained by sizing one or both faces of the jute or similar fibrous web with a sizing composition 3 containing a 10 heat insulating material which is preferably zonolite or some other exfoliated vermiculite or rock wool or some other fireproof insulator. The zonolite or other fire-resistant, heat insulator is incorporated in a mixture or emulsion of a suitable 15 binder such as latex, bentonite and water. The zonolite or other fire-resistant, heat insulator is comminuted and may vary in fineness so that it will pass through a screen ranging from ten to one hundred mesh, that is, having from ten 20 to one hundred openings per square inch of screen. The jute fiber mat or mat made from the other above-mentioned fibrous materials is then sized on one or both sides by dipping or otherwise treating with the above-mentioned sizing. Upon drying the sizing becomes stiff and 25 stiffens and rigidifies the jute fiber mat thus making a board. If the board is to be used other than on flat surfaces, the jute mat, subsequent to sizing and before the size dries, is placed in 30 a suitable form corresponding to the contour of the dash, for example, and the sizing permitted to dry. After drying, the thus sized jute board will conform to the contour of the dash or other 35 surface upon which it is used.

40 Aside from rigidifying and making a board out of the jute fiber mat, the zonolite or other sizing makes the board fire-resisting and heat insulating.

45 A jute fiber mat sized on one or both surfaces with a zonolite sizing, upon drying to form a board, can be used for heat and sound insulating the vehicle body dash as effectively and efficiently as the above-mentioned heat and sound insulating assembly presently being used comprising the jute fiber mat, compressed wood fiberboard, and decorative fiber asphalt composition board.

55 This jute fiber or other soft felted board hav-

ing the zonolite sizing can be embossed while wet with any desirable surface ornamentation and colored to suit the individual requirements of the user.

- 5 After the woven fabric or felted jute web is sized and the sizing dried, a board is formed consisting of three layers or plies, an inner layer of jute between two stiff outer layers consisting principally of zonolite bound to the jute.
- 10 The jute inner layer remains compressible and soft and thus retains its sound insulating properties and the dry sizing which has penetrated the jute fibers adjacent the surface of the jute inner layer, integrates these outer fibers and
- 15 forms one or two spaced outer layers which serve as stiffeners and cooperate to make the resultant board self-supporting. However, the resultant board is bendable and flexible. Upon being bent or twisted, the jute inner layer, owing
- 20 to its compressibility or distortability, permits relative movement between the outer layers of zonolite or other sizing.

I claim:

1. An automotive vehicle dash heat and sound insulator comprising an inner layer of a limp, non-self-sustaining fibrous material forming a sound insulator, and a rigidifying coating on one 5 or both faces of the fibrous material of comminuted exfoliated vermiculite, and a binder for binding the comminuted exfoliated vermiculite to itself and the fibrous layer.

2. A fire-resistant, heat and sound insulating 10 board comprising a compressible, limp inner layer of fibrous material and a coating for one or both of the faces of the inner layer of a sizing comprising comminuted exfoliated vermiculite bound to, and impregnating the outer surfaces of the 15 inner fiber layer, and a binder for binding the comminuted exfoliated vermiculite to the inner layer, the said sizing coating on the outer face of the fibrous inner layer serving as a stiffener to make the board self-sustaining. 20

WILLIAM N. MAYO.